

# United States Patent Office

2,725,286

Patented Nov. 29, 1955

1

2,725,286

## ABRASIVE AND GRINDING WHEEL

Loring Coes, Jr., Brookfield, Mass., assignor to Norton Company, Worcester, Mass., a corporation of Massachusetts

No Drawing. Application March 10, 1953,  
Serial No. 341,595

4 Claims. (Cl. 51—298)

The invention relates to abrasives and grinding wheels. One object of the invention is to provide a superior grinding wheel for snagging operations. Another object of the invention is to provide a grinding wheel suitable for use in a power controlled billet grinder. In this connection billet grinding has heretofore been done principally with so-called swing frame grinders in which the operator had to move and control the wheel by his own physical strength. Weights were used to give the grinding pressure but the resultant forces had to be counteracted by the operator's strength. Recently power operated billet grinders have been developed in which the operator merely moves valves or the like to move the grinding wheel to different parts of the billet and, since the force to move the grinding wheel is hydraulic, great pressures can be used. Such machines are described in pending applications of my colleague George Comstock, 3rd, Serial No. 285,423, filed May 1, 1952, and Serial No. 287,530, filed May 13, 1952, also in copending applications of my colleague Carl Soderlund, Serial No. 304,170, filed August 13, 1952, and Serial No. 312,715, filed October 2, 1952.

Another object of the invention is to provide a grinding wheel capable of being used at very high speeds, that is to say having a breaking strength as measured in surface feet per minute materially higher than billet grinding wheels or other wheels of this general type heretofore made. Another object of the invention is to provide a grinding wheel, for use for example as a billet grinding wheel, which can be used at high pressures and under such conditions to give superior grinding results as measured in the conventional manner.

Other objects will be in part obvious or in part pointed out hereinafter.

I have found that an abrasive, superior to fused alumina for some purposes, can be made by the following process:

Calcined bauxite is ball milled 10 to 20 hours in a steel ball mill. The fine powder is then stirred into 10% hydrochloric acid and agitated for about 10 hours. The acid is decanted and the sludge washed free of acid. The sludge is dried to about 2% water. The nearly dry powder is screened and pressed into bricks at about 2500 pounds per square inch. The bricks are dried completely and fired at 1600° C. for 2 to 5 hours. The black bricks are then crushed down and screened for the desired abrasive sizes.

The abrasive grain thus produced has a composition which varies according to the analysis of the bauxite but which will be within the limits shown in the following table.

TABLE I

|                                     | Percentage range, by weight |
|-------------------------------------|-----------------------------|
| Alumina, $Al_2O_3$                  | 65.0 to 97.0                |
| Silica, $SiO_2$                     | .3 to 16.0                  |
| Iron oxide, calculated as $Fe_2O_3$ | 4.0 to 35.0                 |
| Titania, $TiO_2$                    | 0.0 to 12.0                 |
| Lime, $CaO$                         | 0.0 to 1.5                  |
| Magnesia, $MgO$                     | 0.0 to 1.0                  |
| Other compounds or elements         | Less than 2                 |

2

This abrasive grain is characterized by having fine crystalline structure, great strength and a hardness nearly equal to the hardest fused alumina. Its outstanding quality is its strength which is surprisingly greater than that of any fused alumina; this may be due to the fineness of the crystal structure. The strength is probably also increased by the fact that the iron oxide includes a large proportion of magnetite,  $Fe_3O_4$ . There is substantially no water of crystallization left in the material; bauxite as mined contains a large proportion of water of crystallization.

A further surprising matter is that this abrasive made as described and having the composition of Table I can be used to make phenolic resinoid bonded grinding wheels having a materially higher breaking speed than wheels made out of regular fused alumina, the standard abrasive for billet snagging up to now. It is known that the breaking speed for a grinding wheel given in surface feet per minute is substantially independent of the diameter when the central hole is relatively small as is the case with snagging wheels. Hot pressed phenolic resin bonded snagging wheels of hard grades made in a standard manner and having the standard regular alumina abrasive had a breaking speed of from 20,000 surface feet per minute to 22,000 surface feet per minute. Exactly similar hot pressed phenolic resin bonded snagging wheels of the same hard grades made in the same standard manner and having the sintered calcined bauxite abrasive of Table I had a breaking speed of from 28,000 surface feet per minute to 30,000 surface feet per minute.

For comparison with the calcined sintered bauxite of Table I, I provide analyses of some lots of recently produced regular fused alumina.

TABLE II

|                       | Percentages, by Weight |        |       |       |        |       |
|-----------------------|------------------------|--------|-------|-------|--------|-------|
|                       | Lot A                  | Lot B  | Lot C | Lot D | Lot E  | Lot F |
| 40                    |                        |        |       |       |        |       |
| Alumina, $Al_2O_3$    | 93.50                  | 93.60  | 93.50 | 93.50 | 93.51  | 93.60 |
| Silica, $SiO_2$       | 1.85                   | 1.91   | 1.91  | 1.87  | 2.11   | 1.88  |
| Iron oxide, $Fe_2O_3$ | 0.18                   | 0.16   | 0.14  | 0.14  | 0.11   | 0.13  |
| Titania, $TiO_2$      | 3.32                   | 3.30   | 3.42  | 3.42  | 3.44   | 3.31  |
| Lime, $CaO$           | 0.13                   | 0.13   | 0.11  | 0.09  | 0.11   | 0.13  |
| Magnesia, $MgO$       | 0.38                   | 0.32   | 0.34  | 0.32  | 0.31   | 0.35  |
| Zirconia, $ZrO_2$     | 0.47                   | 0.58   | 0.51  | 0.49  | 0.42   | 0.40  |
|                       | 99.81                  | 100.00 | 99.93 | 99.83 | 100.01 | 99.80 |

The following tables give analyses of typical bauxites found in various parts of the world excluding, however, the water of crystallization. These tables therefore approximately show the composition of various calcined bauxites all of which can be used in this invention. It will be noted that the percentages do not add up exactly to 100, but they come close and the differences represent minor errors of analysis and calculation. Furthermore evidently many of the samples were not analyzed for  $CaO$  or  $MgO$  but doubtless all of them contained a small amount thereof.

TABLE III

Analysis of five different lots of calcined bauxite

|                                  | Percentages, by Weight |        |        |       |       |       |
|----------------------------------|------------------------|--------|--------|-------|-------|-------|
|                                  | Lot 1                  | Lot 2  | Lot 3  | Lot 4 | Lot 5 |       |
| 65                               |                        |        |        |       |       |       |
| Alumina, $Al_2O_3$               | 89.75                  | 77.50  | 97.00  | 94.90 | 96.00 |       |
| Silica, $SiO_2$                  | 2.89                   | 14.10  | .93    | 4.03  | 1.36  |       |
| Iron Oxide, calculated $Fe_2O_3$ | 2.40                   | 8.46   | .42    | .74   | 1.08  |       |
| Titania, $TiO_2$                 | 5.06                   |        | 1.57   | .15   | 1.49  |       |
| Lime, $CaO$                      |                        |        |        |       |       |       |
| Magnesia, $MgO$                  |                        |        |        |       |       |       |
|                                  | Total                  | 100.10 | 100.06 | 99.92 | 99.82 | 99.93 |
| 70                               |                        |        |        |       |       |       |

TABLE IV  
*Analysis of five different lots of calcined bauxite*

|                                                      | Percentages, by Weight |       |        |       |        |
|------------------------------------------------------|------------------------|-------|--------|-------|--------|
|                                                      | Lot 6                  | Lot 7 | Lot 8  | Lot 9 | Lot 10 |
| Alumina, $\text{Al}_2\text{O}_3$ .....               | 81.50                  | 85.10 | 83.20  | 91.50 | 82.75  |
| Silica, $\text{SiO}_2$ .....                         | 1.60                   | 1.97  | .37    | 2.44  | .75    |
| Iron Oxide, calculated $\text{Fe}_2\text{O}_3$ ..... | 3.57                   | 3.63  | 7.35   | 3.22  | 14.50  |
| Titania, $\text{TiO}_2$ .....                        | 11.90                  | 8.65  | 9.18   | 2.69  | 1.99   |
| Lime, $\text{CaO}$ .....                             | 1.11                   | trace | trace  | trace | trace  |
| Magnesia, $\text{MgO}$ .....                         | .41                    | .52   | trace  | trace | trace  |
| Total.....                                           | 100.09                 | 99.87 | 100.10 | 99.85 | 99.99  |

TABLE V  
*Analysis of five different lots of calcined bauxite*

|                                                      | Percentages, by Weight |        |        |        |        |
|------------------------------------------------------|------------------------|--------|--------|--------|--------|
|                                                      | Lot 11                 | Lot 12 | Lot 13 | Lot 14 | Lot 15 |
| Alumina, $\text{Al}_2\text{O}_3$ .....               | 66.25                  | 89.30  | 69.50  | 75.00  | 67.95  |
| Silica, $\text{SiO}_2$ .....                         | .90                    | .94    | .33    | 15.90  | 1.69   |
| Iron Oxide, calculated $\text{Fe}_2\text{O}_3$ ..... | 29.83                  | 5.62   | 29.60  | 4.86   | 27.00  |
| Titania, $\text{TiO}_2$ .....                        | 3.18                   | 4.10   | .91    | 2.81   | 3.45   |
| Lime, $\text{CaO}$ .....                             | .....                  | .....  | .....  | .....  | .....  |
| Magnesia, $\text{MgO}$ .....                         | .....                  | .....  | .....  | .....  | .....  |
| Total.....                                           | 100.16                 | 99.96  | 100.34 | 98.57  | 100.09 |

TABLE VI  
*Analysis of five different lots of calcined bauxite*

|                                                      | Percentages, by Weight |        |        |        |        |
|------------------------------------------------------|------------------------|--------|--------|--------|--------|
|                                                      | Lot 16                 | Lot 17 | Lot 18 | Lot 19 | Lot 20 |
| Alumina, $\text{Al}_2\text{O}_3$ .....               | 72.50                  | 65.20  | 65.40  | 68.30  | 85.50  |
| Silica, $\text{SiO}_2$ .....                         | .88                    | 1.12   | 3.16   | 9.20   | 4.26   |
| Iron Oxide, calculated $\text{Fe}_2\text{O}_3$ ..... | 23.60                  | 33.60  | 28.80  | 21.61  | 4.51   |
| Titania, $\text{TiO}_2$ .....                        | 3.10                   | 1.44   | .....  | .....  | 5.00   |
| Lime, $\text{CaO}$ .....                             | .....                  | .....  | .....  | .35    | .....  |
| Magnesia, $\text{MgO}$ .....                         | .....                  | .....  | .....  | .43    | .....  |
| Total.....                                           | 100.08                 | 99.92  | 98.80  | 99.89  | 99.27  |

Bauxite, as mined, contains a large proportion of water of crystallization. The various bauxites whose analyses are given in Tables III, IV, V and VI, Lots 1 to 20 inclusive, had originally from about 10% to about 33% of water which, however, was driven off by the calcining process so that these tables give analyses of the calcined bauxite. Bauxite, as mined and also after calcination, contains some iron oxide, as given in the tables. But this is different iron oxide from the iron oxide of the regular fused alumina (Table II). In the bauxite a large percentage (at least one half) of the total iron oxide is magnetite,  $\text{Fe}_3\text{O}_4$ . In the pigs of regular fused alumina there is present iron oxide  $\text{Fe}_2\text{O}_3$  and also some magnetite,  $\text{Fe}_3\text{O}_4$ , and also some elementary iron; the magnetite  $\text{Fe}_3\text{O}_4$  and the iron are, however, removed in the magnetic separating process, so that the final abrasive material contains substantially none thereof. Table II reports the analyses of six lots of regular fused alumina abrasive from which the magnetite and the free iron have been eliminated.

Thus the abrasive used in this invention is calcined bauxite which has never been fused, but which has been sintered at a temperature of at least 1550°C., for at least two hours. It can be sintered at higher temperatures and for a longer time provided it is never fused (melted).

The abrasive according to this invention is not corundum under another name (e. g. Upper Hessian bauxite). Corundum is an abrasive which is used for the manufacture of grinding wheels without being sintered. The steps of grinding (ball milling) the bauxite into fines and then pressing the fines into bricks are important steps without which, or the equivalent, the abrasive of

this invention cannot be produced. These steps permit the sintering to produce fine grained strong bricks (of substantial size, e. g. 6" x 3" x 2") which are later crushed to produce the abrasive particles.

5 The manufacture of phenolic resin bonded grinding wheels out of abrasive has been abundantly described and is well known. I prefer to make hot pressed wheels for billet grinding operations; this is done by thoroughly mixing reactive phenol-formaldehyde powdered resin with the abrasive, placing the mixture in a mold, and pressing while heating to resin curing temperature which is usually around 175°C. Steam heated hot presses are used. Such wheels have very low porosity, around 2% or less. They can be described as wheels consisting of abrasive bonded 10 with thermo-irreversible phenol formaldehyde resin. Fillers can and preferably will be used; such fillers in the form of fines are simply mixed with the resin and abrasive prior to loading the mold. Typical fillers are cryolite, iron pyrites and potassium fluoborate; the latter two are frequently used in combination. See U. S. Patents Nos. 2,308,981; 2,308,983; and 2,408,319.

A practical test of the quality of a grinding wheel is to square the amount of material removed in pounds and to divide this square by the loss of the wheel by wear 15 measured in cubic inches. A number results which is known as the quality number, and the more economical the wheel (taking into consideration the operator's pay, shop overhead and cost of the wheel) the higher the quality number. The comparison is made between wheels 20 of the same size, and of the same ingredients in the same proportions except for one variable being evaluated. Grinding tests on wheels according to the invention operated at high surface speeds (peripheral velocities) and great pressure gave quality numbers as high as 75. The 25 quality number of the best similar wheels made out of regular fused alumina abrasive (Table II) at the highest commercial speed and highest commercial pressure is from 35 to 40. This is when using the hand controlled snagging machines referred to as swing frame grinders. 30 This quality number of the old regular fused alumina wheels could, by increasing the pressure to a certain value, be raised to 50. Raising the pressure above that certain value caused excessive wheel wear which lowered the quality number. It has already been pointed out that 35 the wheels of the invention can be run at higher speeds than would be safe for wheels formerly made. Thus wheels according to the invention will give superior performance in the power operated and controlled billet grinders previously referred to.

#### EXAMPLE I

Two wheels each sixteen inches in diameter by two and one-half inches thick with six inches diameter central holes were molded in a hot press for one hour at about 40 two and one-half tons per square inch and at 160°C. temperature. The wheels were then removed from the press and from the molds and were baked in an oven at 45 temperatures rising from room temperature to 140°C. in four hours then at 140°C. for eighteen hours. These 50 wheels were made from a mixture of the calcined sintered bauxite above described, in a mixture of particles of from No. 12 to No. 16 grit sizes, reactive powdered phenol 55 formaldehyde resin of the brand BR 2417 or equivalent, and fillers, in the proportion of 54 volume percent abrasive, the remainder bond and fillers. The wheels had no pores. Of the 46 volume percent bond and fillers there was 55 volume percent of phenol formaldehyde resin, 21 volume percent iron pyrites, 21 volume percent potassium fluoborate and 3 volume percent lime,  $\text{CaO}$ . The iron 60 pyrites and the potassium fluoborate  $\text{KBF}_4$  are grinding promoting agents, the  $\text{CaO}$  is a dehydrating agent eliminating the water liberated during curing.

The wheels of Example I were (successively) mounted 65 in the snagging grinder of U. S. application Serial No. 285,423 above referred to and used to grind stainless steel, 70 all grinding being done on steel of the same composition 75

and physical characteristics. The wheels were marked 1 and 2 for identification although they were exactly alike so far as it was possible to make them. In the following table is given the results of the grinding tests, at different wheel speeds as measured in surface feet per minute, where the left hand column identifies the wheel, the next column gives the peripheral velocity in surface feet per minute, the next column gives the pressure between the wheel and the steel in pounds, the next column gives the wheel wear in total cubic inches lost, the next column gives the steel removed in total pounds, and the right hand column gives the quality number to the nearest integer derived by squaring the material removed in the above units and dividing this square by the wheel wear in the above units.

TABLE VII  
*Grinding results*

| Wheel Number | Peripheral Speed | Pressure | Wheel Wear | Material Removed | Quality Number |
|--------------|------------------|----------|------------|------------------|----------------|
| 1-----       | 9,500            | 200      | 5.0        | 6.2              | 8              |
| 2-----       | 9,500            | 200      | 4.8        | 6.3              | 8              |
| 1-----       | 12,400           | 200      | 6.4        | 10.2             | 16             |
| 2-----       | 12,400           | 200      | 8.0        | 12.3             | 19             |
| 1-----       | 12,400           | 350      | 18.9       | 27.2             | 39             |
| 2-----       | 12,400           | 350      | 20.0       | 28.3             | 40             |
| 1-----       | 12,400           | 480      | 126.0      | 97.5             | 75             |
| 2-----       | 12,400           | 480      | 156.0      | 108.0            | 75             |

The figures in Table VII were based upon four fifteen minute grinding tests except for the last (bottom) two. The next to last (next to bottom) figures are based upon one fifteen minute test and the last (bottom) figures are based upon one twelve minute test. The reason for shortening the test at the end is that the wheels had been considerably reduced in diameter and below a certain size grinding is difficult.

In general usually more than fifty percent of the iron oxide in the abrasive of the invention is magnetic iron oxide,  $Fe_3O_4$ , but the iron oxide is calculated as  $Fe_2O_3$  as is conventional. Fused alumina with the iron and most of the iron oxide removed has a hardness about that of sapphire, which hardness is stated as 9 on Mohs' scale by definition according to Mohs.

It will thus be seen that there has been provided by this invention an abrasive and a grinding wheel in which the various objects hereinabove set forth together with many thoroughly practical advantages are successfully achieved. As many possible embodiments may be made of the above invention and as many changes might be made in the embodiments above set forth, it is to be understood that all matter hereinbefore set forth is to be interpreted and not in a limiting sense.

I claim:

1. A grinding wheel consisting of abrasive consisting of sintered material derived from calcined bauxite reduced to a fine powder, pressed into masses and sintered at 1550° C. for at least two hours, said abrasive having a composition of

|                                             | Percentage range, by weight |
|---------------------------------------------|-----------------------------|
| Alumina, $Al_2O_3$ -----                    | 65 to 97                    |
| Silica, $SiO_2$ -----                       | .3 to 16                    |
| 10 Iron oxide calculated as $Fe_2O_3$ ----- | 4 to 35                     |
| Titania, $TiO_2$ -----                      | up to 12                    |
| Lime, $CaO$ -----                           | up to 1.5                   |
| Magnesia, $MgO$ -----                       | up to 1                     |
| Other compounds or elements-----            | less than 2                 |
| 15 Water of crystallization-----            | substantially none.         |

said abrasive having a hardness close to 9 on Mohs' scale and a fine crystal structure and having a strength greater than that of fused alumina, said abrasive being bonded with thermo-irreversible phenol formaldehyde resin.

2. A grinding wheel according to claim 1 having a porosity of less than 2%.

3. A grinding wheel consisting of abrasive consisting of sintered material derived from calcined bauxite reduced to a fine powder, pressed into masses and sintered at 1550° C. for at least two hours, said abrasive having a composition of

|                                          | Percentage range, by weight |
|------------------------------------------|-----------------------------|
| Alumina, $Al_2O_3$ -----                 | 65 to 97                    |
| Silica, $SiO_2$ -----                    | .3 to 16                    |
| Iron oxide calculated as $Fe_2O_3$ ----- | 4 to 35                     |
| Titania, $TiO_2$ -----                   | up to 12                    |
| Lime, $CaO$ -----                        | up to 1.5                   |
| Magnesia, $MgO$ -----                    | up to 1                     |
| 35 Other compounds or elements-----      | less than 2                 |
| Water of crystallization-----            | substantially none          |

said abrasive having a hardness close to 9 on Mohs' scale and a fine crystal structure and having a strength greater than that of fused alumina, the major portion of the iron oxide in the abrasive being magnetic iron oxide,  $Fe_3O_4$ , said abrasive being bonded with thermo-irreversible phenol formaldehyde resin.

4. A grinding wheel according to claim 3 having a porosity of less than 2%.

References Cited in the file of this patent

UNITED STATES PATENTS

|              |                   |                |
|--------------|-------------------|----------------|
| 50 2,256,528 | Rowe et al. ----- | Sept. 23, 1941 |
| 2,278,442    | Heany -----       | Apr. 7, 1942   |
| 2,311,228    | Heany -----       | Feb. 16, 1943  |
| 2,363,146    | Roble -----       | Nov. 21, 1944  |
| 2,441,534    | Norton -----      | May 11, 1948   |